

BEST AVAILABLE COPY

Nov. 4, 1924.

1,514,102

R. ROBINSON

PROCESS OF TREATING METAL

Filed Dec. 6, 1920



Inventor  
Richard Robinson  
By H. L. Fitch, Brook Met.

Atty's.

Patented Nov. 4, 1924.

1,514,102

## UNITED STATES PATENT OFFICE.

RICHARD ROBINSON, OF MASURY, OHIO.

## PROCESS OF TREATING METAL.

Application filed December 6, 1920. Serial No. 428,579.

*To all whom it may concern:*

Be it known that I, RICHARD ROBINSON, a citizen of the United States, residing at Masury, in the county of Trumbull and

5 State of Ohio, have invented a certain new and useful Improvement in Processes of Treating Metal, of which the following is a full, clear, and exact description, reference being had to the accompanying drawings.

10 As is well known to those familiar with the art of manufacturing iron and steel, a large percentage of the ingots made from metal recovered from open-hearth and other like furnaces are imperfect because of the 15 "piping" and segregation of the ingots, because of the presence of impurities such as sulphur and phosphorus in a detrimental proportion, and because of the uneven distribution of the cleansing, alloying, or modifying agents in and throughout the iron or steel; furthermore, a large proportion of the 20 finished metal from such furnaces is unsuitable for use because of the presence of seams therein.

25 The general objects of this invention are to provide a process whereby impurities such as the sulphur and phosphorous constituents of the molten mass may be completely and quickly removed and whereby the 30 cleansing, alloying, or other modifying agents may be quickly and uniformly incorporated with the metal, with the result that I am enabled, not only to produce metal which is uniform or homogeneous throughout its mass and which is free from the objections above noted, but to produce the same in a much shorter period of time than is required for the production of the less perfect metal of commerce. I accomplish 35 the objects and results referred to in and through an apparatus such as shown in the drawings forming a part hereof, wherein Fig. 1 represents a central transverse sectional view through a furnace capable of 40 realizing my invention; Fig. 2 a sectional plan view of said furnace; and Fig. 3 a diagrammatic view of the electrical apparatus employed in connection with the furnace shown in the preceding views.

45 50 Describing the various parts by reference characters, 1 denotes the bottom, 2 the sides, 3 the ends, and 4 the top of a furnace of the open-hearth type, the bottom being provided with a lining 5 of ganister or other heat 55 resisting material. The furnace is provided with the tap hole 6 for the removal of

metal and with chambers 7 in the ends thereof for the purpose of heating air and delivering the same above the bath in conjunction with gas or oil burners 18.

60 Projecting downwardly into the furnace chamber 9 are a plurality of heat-resistant tubes 10. Four such tubes are shown as mounted two in each of the sides of the chamber and projecting downwardly and toward the center of the hearth. Adjustably mounted in each of the tubes 10 is an electrode 11, the said electrodes being shown as connected in pairs to electrical conductors 12 extending from opposite sides of a generator 13.

65 Embedded within the bottom wall of the furnace (which may be of magnesite brick) are a plurality of electro-magnets, four which magnets being shown and comprising each 70 a circular core 14 having a winding 15 therearound. These magnets are so arranged that, when the electrodes 11 are in their inwardly adjusted positions, the lower end of each electrode will be above the center 75 of a magnet.

80 With the parts constructed and arranged as described the furnace will be charged in the usual manner, with the electrodes 11 elevated within their respective tubes. The charge may comprise the ordinary pig iron, scrap iron and limestone and, if desired, one or more modifying agents, such as an alloy or alloys or a scavenging agent. The chamber 9 and the charge will be heated by means 85 of the gas or oil burners 18 until the metal is melted—in part at least—and a protecting coating of slag is formed on top of the metal. The supply of fuel to the burners will then be cut off and the electrodes inserted beneath the slag and into the metal, and preferably with their lower ends close to the bottom of the latter and in proximity to one another, as indicated in Figs. 1 and 90 2. Current will then be turned on to the electrodes, current also being supplied to the windings of the electro-magnets. After the current has been turned on to the electrodes, a scavenging agent (such as spiegel-eisen), a degasifying agent (such as fluor spar) or a deoxidizing agent (such as a nitrate) or a combination or combinations thereof may be added to the metal. The electro-magnets cause the current between the electrodes to be deflected, producing a 95 whirling or vortex motion in such current as well as in the molten metal, as indicated

100 105 110

BEST AVAILABLE COPY

1,514,102

at 16 in Figs. 2 and 3. This diffuses quickly throughout the entire mass of molten metal the heat produced by the current and kneads and kilns the metal.

5 Some, at least, of the impurities are quickly reduced to a gaseous condition by this action. The molten scavenger acts as an electrolyte and affords a whirling path of least resistance along which at least some 10 of the gaseous impurities move and by which they are delivered to the appropriate electrodes, rising along such electrodes and being caught and held by the slag, together with other impurities which have been carried along by such gas, the scavenger by this time having been gasified and caught by the slag.

During this operation, the metal is protected from oxidation by the slag coating 20 on the top thereof, while heated internally at the bottom of the furnace by the electrodes. This location of electrodes prevents any adhesion of metal to the bottom of the furnace or to the electrodes.

25 This mode of treatment enables any limestone and other ingredients that may be at the bottom of the furnace to be quickly raised, and quickly liberates impurities in a gaseous form; the said impurities being 30 collected by the slag; and, where alloying or other modifying agents are employed, insures a rapid and uniform incorporation of the same with the molten metal. All of the gases will be eliminated, thus avoiding 35 "piping" and segregation of the ingots and seams in the metal; and the time required for "making the heat" will not exceed half the time ordinarily required for such purpose.

40 At the end of the heating by the electrodes, the latter are raised out of the bath into their respective tubes and the burners are operated for a short time in order to melt any slag that may have adhered to 45 the sides of the furnace, so as to enable the latter to be tapped.

While I have described my process with reference to the production of iron and steel, I do not propose to limit the scope 50 of my invention to such metals, as the process is not only applicable to but valuable in connection with the treatment of other metals, with such variations in amperage suited to the reduction and refining of such metals, respectively.

Having thus described my invention, what I claim is;

1. The process of treating metal which 60 comprises reducing or melting the metal and maintaining the same in a molten condition by means of heat applied thereto from above, providing a protecting coating of slag for such molten metal, and subjecting the molten metal to the action 65 of an electric current supplied through elec-

trodes operating adjacent to the bottom of the molten mass and beneath the slag coating.

2. The process of treating metal which comprises reducing or melting the metal 70 and maintaining the same in a molten condition by the combustion of gaseous fuel applied thereto from above in a furnace of the open-hearth type, providing the molten metal with a protecting coating of slag, and subjecting the molten metal to the action 75 of an electric current flowing therethrough beneath the slag coating.

3. The process of treating molten metal which comprises forming a protecting coating 80 of slag for such metal and subjecting the metal thus protected to a kneading action by means of an electric current passing therethrough beneath the said coating and adjacent to the bottom of the mass 85 of such metal and in the presence of one or more modifying agents.

4. The process of treating molten metal which comprises providing the same with an oxygen or air-excluding coating and subjecting the metal below such coating to the 90 action of electrical heating means operating adjacent to the bottom of the metal mass below the said coating and operating to stir and knead the molten metal 95 charge.

5. The process of treating molten metal which comprises providing the same with an oxygen or air-excluding coating and subjecting the metal below such coating to the 100 action of electric current supplied through the metal by electrodes operating adjacent to the bottom of the metal mass.

6. The process of treating molten metal in a furnace which comprises providing a 105 mass of such metal with an air or oxygen-excluding coating, and subjecting the molten mass below such coating to the action of an electric current supplied therethrough by electrodes located within and adjacent 110 to the bottom of such mass, whereby adhesion of such metal to the bottom of the furnace or to the electrodes is prevented and the molten metal charge is kneaded.

7. The process of treating metal which 115 comprises preliminarily fusing such metal with slagging material to provide a protecting coating of slag, supplying electric current to and between electrodes extending into the metal below such coating and through the metal interposed between such electrodes, and imparting to the current flowing through such mass a whirling motion whereby the mass is kneaded and rendered uniform in composition.

8. The process of treating metal which 120 comprises preliminarily fusing such metal with slagging material to provide a protecting coating of slag, supplying electric current to and between electrodes extending 125 130

- into the metal below such coating and through the metal interposed between such electrodes, and subjecting the current flowing through such mass to the action of an 5 electro-magnet, whereby the current is deflected and the mass is kneaded and rendered uniform in composition.
9. The process of treating metal which comprises preliminarily fusing the upper 10 portion of a charge of such metal with slag producing material, thereby to produce a protecting coating of such slag, supplying electric current to and between electrodes extending into the metal below such coating 15 and through the metal interposed between such electrodes, and subjecting the current thus supplied to the action of magnetic excitation, thereby to impart a whirling motion to the current in such metal and to the 20 metal itself.
10. The process of treating metal which comprises providing the same with a protecting coating of slag, supplying electric current to and between electrodes extending 25 into the metal below such coating and through the metal interposed between such electrodes, in the presence of a scavenger, and subjecting the current thus supplied to the action of magnetic excitation, thereby to 30 impart a whirling motion to the current in such metal and to the metal itself.
11. The process of treating metal which comprises providing the same with a protecting coating of slag, subjecting the mass 35 of metal beneath such coating to the action of electricity supplied at the bottom of the metal mass through electrodes and in the presence of a scavenger, and subjecting the current passing between such electrodes and 40 through the metal to the action of one or more electro-magnets thereby to deflect such current and impart a whirling motion thereto and to the molten metal.
12. The process of treating metal which comprises providing the same with a protecting coating of slag, supplying electric current to and between electrodes extending 45 into the mass of metal below such coating and through the metal interposed between such electrodes in the presence of a scaveng- 50 ing agent and a degasifying agent, and subjecting the current thus supplied to the action of one or more electro-magnets serving to deflect the current and to produce a 55 whirling motion in the same and in the molten metal.
13. The process of treating metal which comprises providing the same with a protecting coating of slag, supplying electric current to and between electrodes extending 60 into the mass of metal below such coating and through the metal interposed between such electrodes in the presence of one or more modifying agents, and discharging impurities in the form of gases along one or 65 more of said electrodes.
14. The process of treating molten metal which comprises providing the same with a protecting coating of slag, and supplying electric current to and between electrodes 70 extending into the mass of metal below such coating and through the metal interposed between such electrodes in the presence of deoxidizing and degasifying agents, whereby the impurities are discharged in the 75 form of gases along one or more of said electrodes.

In testimony whereof, I hereunto affix my signature.

RICHARD ROBINSON.